

# United States Patent Office

2,885,752

Patented May 12, 1959

1

2,885,752

## METHOD OF PRODUCING A FULLY-KILLED STEEL WITH RIMMING CHARACTERISTICS

Dennis J. Carney, Chicago, Ill., assignor to United States Steel Corporation, a corporation of New Jersey

No Drawing. Application April 26, 1954  
Serial No. 425,757

8 Claims. (Cl. 22—216)

This invention relates to the production of fully-killed steels and more particularly to austenitic-chromium-manganese fully-killed steels having improved characteristics resulting from the evolution of gas therefrom after teeming.

The chemical characteristics of the alloying elements involved and economical considerations make it very desirable to make all high-alloy and most alloy steels following conventional practice of fully killing them, i.e. fully deoxidizing the metal by adding to it appropriately selected elements, such as aluminum and silicon, having a greater affinity for oxygen than iron. Such elements combine with oxygen dissolved in iron forming compounds largely incapable of taking part in any subsequent reactions. Thus no gas is evolved when a killed steel solidifies after teeming into ingot molds. As a result, during solidification the steel shrinks with the formation of internal shrinkage cavity. Occasionally such pipe may be tolerated, as in making seamless piping or transformer grades silicon steel sheets, but, as a general rule, it must be eliminated somewhere in the processing cycle generally by cropping the ingot.

The usual and most widely used method for accomplishing pipe elimination in killed steels consists in placing above the ingot molds a hot top, namely a container possessing lesser heat abstracting characteristics than the metal of the ingot mold and which permits a portion of the metal, usually 10 to 20%, to remain liquid for a longer time than the body of ingots and to feed molten metal into the pipe cavity produced during solidification.

With the use of properly designed hot tops, all pipe is concentrated therein and is removed by cropping the hot top after the solidification is completed. Cropped hot tops are scrapped which, in case of high-alloy steels, exemplified by stainless, high-speed and similar alloys, causes heavy financial losses.

In certain low-carbon grades of steel, it is common practice to make steel by rimming practice, i.e. with at least sufficient evolution of gas, largely carbon monoxide, during solidification to at least prevent shrinkage and pipe formation during freezing. In addition to permitting use of a very high percentage of the total ingot and the elimination of hot topping, this results in a "rim" of essentially pure steel uncontaminated by the various inclusions appearing in all steels. This rim has very beneficial effects during rolling, since troublesome seams, etc. are largely eliminated. In killed steels due to the "killing" agent combining with the available oxygen, no rimming can take place and such desirable results thereof have hitherto not been obtainable.

It is accordingly an object of this invention to provide a method of forming killed steel ingots having the characteristics of rimmed steels.

It is another object of this invention to eliminate the necessity of hot-topping fully-deoxidized alloy steel ingots.

I achieve the foregoing objects by introducing sufficient inert gas into the metal while molten and prior to teeming to promote a rimming action therein and formation

2

of gas-filled cavities in the metal during its solidification to offset the decreased volume of the metal due to cooling and solidification thereof.

The preferred gas for practicing my invention is nitrogen which I introduce into the molten bath as a solid compound such as nitrogen-bearing salt, cyanamide, or a metallic nitride. While adequate nitration has been recorded with the use of all these additions, the employment of metallic nitrides, particularly of chromium-nitride in case of stainless steels, introduces additional advantages favoring their use. For example, high nitrogen ferro-chromium may be used in chromium alloys or high nitrogen-manganese or ferro-manganese in manganese alloys. Nitrogen may also be added in the form of a gaseous compound, such as ammonia.

A close control of the gas evolution in the present process is possible only when the body of the metal is free from dissolved oxygen capable of generating carbon monoxide on solidification. With this object in view, a thorough killing of the steel to be treated before adding nitrogen-bearing substances is desirable, and can be accomplished in a number of conventional ways such as those hereinbefore mentioned. This complete killing is of course particularly desirable in the high alloy steels such as austenitic-chromium-manganese steels. Neither the kind of deoxidizers used nor the sequence of their addition appear to bear on the efficiency of the present process, provided the deoxidation reaction is properly effected.

It has been found that mere addition of nitrogen to steel, which is well known, cannot accomplish the results contemplated by this invention. In order to be effective, the gas has to be introduced in closely controlled percentages depending, among others, on the composition of the steel treated and teeming method used. It is essential that the amount of nitrogen added should be in excess of the solubility of nitrogen in the particular steel at its melting point. This provides a volume of evolved gas sufficient to impart to the steel the properties ranging from those wherein the shrinkage cavity is merely replaced by numerous voids in a random distribution to those of fully-rimmed steel wherein the evolution of gas from the steel is sufficient to permit the formation of an external rim of pure metal.

Extensive tests have demonstrated that liquid pure iron dissolves a matter of 0.040-0.045% nitrogen at its melting point, and can retain but 0.010-0.015% nitrogen on solidification. This can be stated that the maximum percentage of nitrogen which can be incorporated in pure iron cannot exceed 0.045% nitrogen and that adding more than 0.015% nitrogen to it will cause formation of blow holes in castings on solidification. Other tests have shown a very pronounced difference in solubility of the gas caused by alloying pure iron with other elements, and the digression of this solubility from that expected from the combined effect of individual elements alloyed with the iron.

I have discovered that a proper balancing of gas evolution rate on solidification and the amount of nitrogen added to the molten steel is a function of steel composition and can be expressed by appropriate formulas empirically derived in each individual case.

Taking as an illustration a group of austenitic alloys containing 16-20% chromium, 4-14% manganese, 4%, maximum, nickel and not more than 0.20% carbon, one can use for determining the percentage of nitrogen to be added for the desired gas evolution the formula:

$$\text{Percent Cr} + 1.75 \times \text{percent Mn} + 2 \times \text{percent Ni}$$
$$70 \text{ Percent N} = \frac{\text{Percent Cr} + 1.75 \times \text{percent Mn} + 2 \times \text{percent Ni}}{100}$$

This formula provides a desired minimum nitrogen

concentration for gas evolution without detracting from the austenitic character of the alloys and is accurate, as shown by experiments, within  $\pm 0.05\%$  nitrogen. Three commercial heats of this alloy listed in the following tabulation may serve as an illustration:

| Heat No. | C   | Mn    | P    | S    | Si  | Ni   | Cr    | N <sub>2</sub> | Ferrite at 2,100° F. percent |
|----------|-----|-------|------|------|-----|------|-------|----------------|------------------------------|
| 1        | .10 | 7.00  | .014 | .011 | .36 | 3.61 | 16.78 | .40            | 0                            |
| 2        | .04 | 9.65  | .019 | .006 | .43 | 2.33 | 18.15 | .49            | 0                            |
| 3        | .11 | 11.28 | .018 | .006 | .52 | 0.11 | 17.11 | .44            | 0                            |

These heats were all cast into 23x35x40 inch ingots in bottle-top molds and had sufficient rimming action for a very satisfactory mechanical capping. No particular precautions were taken in their manufacture and no deviations from the conventional good steel-making practice were committed, as it can be seen from the following melting sheet of electric furnace heat 1.

|                                                   |       |
|---------------------------------------------------|-------|
| Began charge, 3100 lbs. slab                      | 8:30  |
| Full power on                                     | 8:40  |
| 100 lbs. light scrap, liquid pool                 | 10:25 |
| 1200 lbs. slabs                                   | 11:15 |
| Began feeding 1410 lbs. low-carbon ferrochrome    | 11:25 |
| 200 lbs. ferrochrome pellets                      | 11:55 |
| 1000 lbs. slabs                                   | 12:00 |
| 150 lbs. nickel                                   | 12:35 |
| 150 lbs. nickel                                   | 12:45 |
| Finish feeding low-carbon ferrochrome             | 12:50 |
| 270 lbs. low-carbon ferromanganese                | 12:50 |
| 580 ferrochrome pellets, power cut                | 1:30  |
| Power full                                        | 1:32  |
| Power cut                                         | 1:38  |
| Began to skim slag                                | 1:45  |
| Full power                                        | 1:54  |
| 380 lbs. electrolytic manganese, violent reaction | 1:55  |
| 100 lbs. pig iron                                 | 2:03  |
| Began tap                                         | 2:17  |
| Tapped                                            | 2:19  |

The scrap used consisted of low-metallocid crops, ferrochromium pellets which analyzed 62.09% chromium, 5.47% silicon, 2.06% nitrogen, 0.11% carbon, and the electrolytic manganese contained 5.81% nitrogen.

The nitrogen content of these alloys was balanced in accordance with the above formula so that the desired volume of gas was evolved at a proper rate on solidification. The ingots produced were essentially austenitic, both at hot-rolling and room temperatures, and their hot workability was good. The physical properties of these ingots were similar, in general, to conventional 17% chromium-7% nickel and 18% chromium-9% nickel alloys, and the elimination of hot tops increased their ingot to slab yield from 70-73% to 80-90%.

Rimming action in other compositions of steel can be obtained by similarly adding sufficient nitrogen to exceed the solubility limit thereof in the particular composition at its melting point. A conventional 17% chromium stainless steel has been made with good rimming action as has the so-called Hadfield manganese steel when treated in accordance with my invention by adding nitrogen above the foregoing solubility limit. By proper experimentation, the above formula can be modified for each such composition.

It must be emphasized that the formula presented is a ready indication of the minimum amount of nitrogen for a particular grade of steel and may require modification for adapting the behavior of the metal to outside conditions, exemplified by dimensions and nature of ingot molds, and for controlling the internal structure of ingots, as when the formation of an external rim of pure metal is to be preferred to a random distribution of voids to offset care of volume reduction. In this latter event

about .03 to .04% more nitrogen is required than is required for making capped chromium-manganese-austenitic steel, for which the formula will determine the proper amount.

While I have shown and described one specific embodiment of my invention, it will be understood that this embodiment is merely for the purpose of illustration and description and that various other forms may be devised within the scope of my invention, as defined in the appended claims.

I claim:

1. A method of making fully deoxidized steel ingots having the dense rim and absence of pipe characteristics of rimmed steel comprising forming a steel melt of the desired composition substantially free from dissolved oxygen, adding nitrogen to said melt in excess of the solubility of nitrogen in said melt at its melting point, then teeming said nitrogen enriched steel melt into ingot molds and permitting it to solidify therein, whereby nitrogen in excess of the amount retainable in the steel in the solid condition evolves as a gas within said melt during solidification thereof, promoting the formation of said rim and preventing the formation of a pipe in the resulting ingots.

2. A method of making fully deoxidized steel ingots having the dense rim and absence of pipe characteristic of rimmed steel comprising forming a steel melt of the desired composition substantially free from dissolved oxygen, adding nitrogen to said melt in excess of the solubility of nitrogen in said melt at its melting point, teeming said nitrogen enriched steel melt into ingot molds, capping said molds and permitting said melt to solidify therein, whereby nitrogen in excess of the amount retainable in the steel in the solid condition evolves as a gas within said melt during solidification thereof, promoting the formation of said rim and preventing the formation of a pipe in the resulting ingots.

3. A method of making fully deoxidized austenitic chromium manganese steel ingots having the dense rim and absence of pipe characteristic of rimmed steel comprising forming a melt of steel containing 16 to 20% chromium, 4 to 14% manganese, 4% maximum nickel, up to .20% carbon and free from dissolved oxygen, adding nitrogen to said melt in excess of the solubility of nitrogen in said melt at its melting point, then teeming said nitrogen enriched steel melt into ingot molds, and permitting it to solidify therein, whereby nitrogen in excess of the amount retainable in the steel in the solid condition evolves as a gas within said melt during solidification thereof, promoting the formation of said rim and preventing the formation of a pipe.

4. A method of making fully deoxidized austenitic chromium manganese steel ingots having the dense rim and absence of pipe characteristic of rimmed steel comprising forming a melt of steel containing 16 to 20% chromium, 4 to 14% manganese, 4% maximum nickel, up to .20% carbon and free from dissolved oxygen, adding nitrogen to said melt in accordance with the formula

$$\text{Percent Cr} + 1.75 \times \text{Percent Mn} + 2 \times \text{Percent Ni}$$

$$60 \text{ Percent N} = \frac{100}{}$$

then teeming said nitrogen enriched steel melt into ingot molds, capping said molds and permitting said melt to solidify, whereby nitrogen in excess of the amount retainable in the steel in the solid condition evolves as a gas within said melt during solidification thereof, promoting the formation of said rim and preventing the formation of a pipe.

5. The process of producing a sound, iron base, stably austenitic alloy containing as necessary elements from ten to thirty percent of chromium, five to twenty percent of manganese and from three tenths to one percent of nitrogen and in which the austenitizing elements and the ferrite forming elements are proportioned to permit a stably austenitic alloy at the desired nitrogen level com-

prising producing a melt of the desired composition, casting the melt into an ingot mold, permitting a solid skin to form on the ingot with the simultaneous ebullition of nitrogen, capping the ingot to entrap a substantial amount of nitrogen in the gaseous form as bubbles, permitting the ingot to completely solidify and subjecting the ingot to intensive hot working whereby the gaseous nitrogen contained in the ingot is redissolved and the sides of the nitrogen cavities welded shut to produce a sound and mechanically strong metal.

6. The process of producing a sound iron base, stably austenitic alloy containing from three tenths of one percent to one percent nitrogen and in which the ferrite forming alloying elements and the austenite forming alloying elements are balanced to produce an alloy which is stably austenitic at room temperature and at the desired nitrogen level comprising establishing a melt of the desired composition, casting the melt into an ingot mold, permitting a solid skin to form on the ingot with the simultaneous ebullition of nitrogen, capping the ingot to entrap a substantial amount of nitrogen in the gaseous form as bubbles, permitting the ingot to completely solidify and subjecting the ingot to intensive hot working whereby the gaseous nitrogen contained in the ingot is redissolved and the sides of the nitrogen cavities welded shut to produce a sound and mechanically strong metal.

7. An ingot of fully deoxidized steel having the dense

rim and absence of pipe characteristic of rimmed steel ingots.

8. An ingot of fully deoxidized austenitic stainless steel having the dense rim and absence of pipe characteristic of rimmed steel ingots.

#### References Cited in the file of this patent

#### UNITED STATES PATENTS

- |    |           |         |       |               |
|----|-----------|---------|-------|---------------|
| 10 | 1,792,967 | Clark   | ----- | Feb. 17, 1931 |
|    | 2,181,693 | Epstein | ----- | Nov. 28, 1939 |
|    | 2,236,504 | Herty   | ----- | Apr. 1, 1941  |

#### OTHER REFERENCES

- |    |                                                                                                                                        |  |  |  |
|----|----------------------------------------------------------------------------------------------------------------------------------------|--|--|--|
| 15 | Section VIII, Sixth Report, Iron and Steel Institute, pages 137-149 relied on. 1935.                                                   |  |  |  |
|    | The Making, Shaping and Treating of Steel, U.S. Steel (6th ed.) 1951. Pages 571-573 and 443-445 relied on.                             |  |  |  |
|    | Section V, Seventh Report of Iron and Steel (1937)                                                                                     |  |  |  |
| 20 | Institute on Heterogeneity of Steel Ingots. Pages 139-142 relied on.                                                                   |  |  |  |
|    | The Ingot Phase of Steel Production, 2nd ed., 1942, pp. 22-24 and 43-47 relied on.                                                     |  |  |  |
| 25 | Section IV. Principles Involved in the Making of Rimming Steel. Fourth Report on the Heterogeneity of Steel Ingots, 1932, pages 68-95. |  |  |  |